



US006071654A

# United States Patent [19]

Camp et al.

[11] Patent Number: **6,071,654**  
[45] Date of Patent: **Jun. 6, 2000**

[54] **NONTRANSPARENT TRANSMISSION DISPLAY MATERIAL WITH MAINTAINED HUE ANGLE**

[75] Inventors: **Alphonse D. Camp**, Rochester; **Peter T. Aylward**, Hilton; **Robert P. Bourdelais**, Pittsford, all of N.Y.

[73] Assignee: **Eastman Kodak Company**, Rochester, N.Y.

[21] Appl. No.: **09/154,691**

[22] Filed: **Sep. 17, 1998**

[51] **Int. Cl.<sup>7</sup>** ..... **G03C 1/765**; G03C 1/795; G03C 1/825; G03C 7/32

[52] **U.S. Cl.** ..... **430/11**; 430/502; 430/531; 430/533; 430/534; 430/536; 430/496; 430/950; 430/510

[58] **Field of Search** ..... 430/510, 536, 430/533, 534, 531, 11, 496, 950, 502

## [56] References Cited

### U.S. PATENT DOCUMENTS

3,944,699 3/1976 Mathews et al. ..... 428/220  
4,187,113 2/1980 Mathews et al. ..... 430/533  
4,283,486 8/1981 Aono et al. ..... 430/505  
4,632,869 12/1986 Park et al. ..... 428/315.5  
4,758,462 7/1988 Park et al. ..... 430/213

4,900,654 2/1990 Pollock et al. ..... 430/533  
4,912,333 3/1990 Roberts et al. ..... 250/487.1  
4,977,070 12/1990 Winslow ..... 430/510  
5,055,371 10/1991 Lee et al. ..... 430/126  
5,100,862 3/1992 Harrison et al. ..... 503/227  
5,212,053 5/1993 McSweeney et al. ..... 430/538  
5,244,861 9/1993 Campbell et al. ..... 430/201  
5,387,501 2/1995 Yajima et al. ..... 430/533  
5,389,422 2/1995 Okazaki et al. ..... 428/141  
5,466,519 11/1995 Shirakura et al. ..... 430/538

### FOREIGN PATENT DOCUMENTS

0 662 633 A1 12/1995 European Pat. Off. .  
WO 94/04961 3/1994 WIPO .

*Primary Examiner*—Richard L. Schilling  
*Attorney, Agent, or Firm*—Paul A. Leipold

## [57] ABSTRACT

The invention relates to a photographic element comprising a translucent base and a color forming layer comprising at least one silver halide emulsion layer and dye forming coupler, wherein said base comprises at least one polymer sheet comprising a transparent polymer sheet containing voids, with the proviso that said translucent sheet is substantially free of white light reflecting pigments and wherein said translucent sheet has a light transmission of between 15% and 85%.

**20 Claims, No Drawings**

**NONTRANSPARENT TRANSMISSION  
DISPLAY MATERIAL WITH MAINTAINED  
HUE ANGLE**

**FIELD OF THE INVENTION**

This invention relates to photographic materials. In a preferred form it relates to a photographic display image.

**BACKGROUND OF THE INVENTION**

It is known in the art that photographic display materials are utilized for advertising, as well as decorative displays of photographic images. Since these display materials are used in advertising, the image quality of the display material is critical in expressing the quality message of the product or service being advertised. Further, a photographic display image needs to be high impact, as it attempts to draw consumer attention to the display material and the desired message being conveyed. Typical applications for display material include product and service advertising in public places such as airports, buses and sports stadiums, movie posters, and fine art photography. The desired attributes of a quality, high impact photographic display material are a slight blue density minimum, durability, sharpness, and flatness. Cost is also important as display materials tend to be expensive compared with alternative display material technology mainly lithographic images on paper. For display materials, traditional color paper is undesirable, as it suffers from a lack of durability for the handling, photoprocessing, and display of large format images.

In the formation of color paper it is known that the base paper has applied thereto a layer of polymer, typically polyethylene. This layer serves to provide waterproofing to the paper, as well as providing a smooth surface on which the photosensitive layers are formed. The formation of a suitably smooth surface is difficult requiring great care and expense to ensure proper laydown and cooling of the polyethylene layers. The formation of a suitably smooth surface would also improve image quality as the display material would have more apparent blackness as the reflective properties of the improved base are more specular than the prior materials. As the whites are whiter and the blacks are blacker, there is more range in between and, therefore, contrast is enhanced. It would be desirable if a more reliable and improved surface for a display material could be formed at less expense.

Prior art photographic reflective papers comprise a melt extruded polyethylene layer which also serves as a carrier layer for optical brightener and other whitener materials, as well as tint materials. It would be desirable if the optical brightener and blue tints, rather than being dispersed in a single melt extruded layer of polyethylene could be concentrated nearer the surface of a display material where they would be more effective optically.

Prior art photographic transmission display materials with incorporated diffusers have light sensitive silver halide emulsions coated directly onto a gelatin coated clear polyester sheet or a gelatin coated clear polyester sheet containing white pigments. Incorporated diffusers are necessary to diffuse the light source used to backlight transmission display materials. Without a light diffuser, the light source would reduce the quality of the image. Typically, white pigments are coated in the bottommost layer of the imaging layers or are added to the polyester sheet. Since light sensitive silver halide emulsions tend to be yellow because of the gelatin used as a binder for photographic emulsions, minimum density areas of a developed image will tend to

appear yellow. A yellow minimum density reduces the commercial value of a transmission display material because the imaging viewing public associates image quality with a white density minimum. It would be desirable if a transmission display material with an incorporated diffuser could have a density minimum with a blue tint, as a blue tinted density minimum is perceptually preferred by the public.

Prior art photographic translucent display materials with incorporated diffusers which include transmission and reflective display materials typically contain some level of white pigment to either diffuse the backlighting source in the case of transmission display materials or provide the desired reflective properties in the case of a reflective display material. While the use of white pigments in display materials does provide the desired diffusion and reflection properties, the white pigments tend to change the hue angle of the color dyes in a developed photographic display image. Dye hue angle is a measure in CIELAB color space of that aspect of color vision that can be related to regions of the color spectrum. For color photographic system there is a perceptual preferred dye hue angle for the yellow, magenta, and cyan dyes. It has been found that when photographic dyes are coated on support containing white pigments, the hue angle of the developed image changes compared to the hue angle of the dyes coated onto a transparent support. The hue angle change of photographic dyes caused by the presence of white pigments often reduces the quality level of the dyes compared to the dye set coated on a transparent base that is substantially free of white pigments. It would be desirable if a developed photographic dye set coated on a translucent support material had a dye hue angle that was not significantly different than the same dye set coated on a transparent support.

Prior art photographic display material use polyester as a base for the support. Typically the polyester support is from 150 to 250  $\mu\text{m}$  thick to provide the required stiffness. A thinner base material would be lower in cost and allow for roll handling efficiency, as the rolls would weigh less and be smaller in diameter. It would be desirable to use a base material that had the required stiffness but was thinner to reduce cost and improve roll handling efficiency.

**PROBLEM TO BE SOLVED BY THE  
INVENTION**

There is a need for a photographic display material that provides less corruption of dye hue angle when coated on a translucent support while, at the same time, provides efficient diffusing of the illuminating light source such that the lighting elements of the light source are not apparent to the viewer.

**SUMMARY OF THE INVENTION**

It is an object of the invention to provide improved photographic display materials.

It is another object to provide photographic translucent display materials that have a maintained dye hue angle.

It is a further object to provide display materials that are low in cost, as well as providing sharp durable images.

These and other objects of the invention are accomplished by a photographic element comprising a base, a color forming layer comprising at least one silver halide emulsion layer and dye forming coupler, wherein said base comprises a translucent polymer sheet comprising a transparent polymer containing voids, wherein said translucent sheet is substantially free of white light reflecting pigments and

wherein said translucent sheet has a light transmission of between 15% and 85%.

In another embodiment, the invention is accomplished by a display apparatus comprising a container provided with one side that is at least partially open or transparent, a light source adapted to provide light directed to the open or transparent side, means to suspend a photographic element comprising a base, a color layer formed by the reaction of at least one silver halide emulsion layer and dye forming coupler, wherein said base comprises a translucent polymer sheet comprising a transparent polymer containing voids, with the proviso that said translucent sheet is substantially free of white light reflecting pigments and said translucent sheet has a light transmission between 15% and 85% and is suspended in said one side that is at least partially open.

#### ADVANTAGEOUS EFFECT OF THE INVENTION

This invention provides brighter, snappy images by maintaining the dye hue of photographic dyes while, at the same time, allowing efficient diffusion of light used to illuminate display materials.

#### DETAILED DESCRIPTION OF THE INVENTION

The invention has numerous advantages over prior art photographic display materials and methods of imaging display materials. The display materials of the invention provide very efficient diffusing of light, while allowing the transmission of a high percentage of the light. These translucent display materials also maintain the dye hue angle of developed photographic dyes when coated on a transparent base. The materials are low in cost, as the translucent polymer sheet is thinner and lower in density compared prior art materials. They are also lower in cost as less gelatin is utilized as no annihilation layer is necessary. The formation of transmission display materials requires a display material that diffuses light so well that individual elements of the illuminating bulbs utilized are not visible to the observer of the displayed image. On the other hand, it is necessary that light be transmitted efficiently to brightly illuminate the display image. The invention allows a greater amount of illuminating light to actually be utilized as display illumination while, at the same time, very effectively diffusing the light sources such that they are not apparent to the observer. The display material of the invention will appear whiter to the observer than prior art materials which have a tendency to appear somewhat yellow as they require a high amount of light scattering pigments to prevent the viewing of individual light sources. These high concentrations of pigments appear yellow to the observer and result in an image that is darker than desirable. These and other advantages will be apparent from the detailed description below.

When referring to the embodiment comprising a biaxially oriented polyolefin sheet laminated to a transparent polymer support, the terms as used herein, "top", "upper", "emulsion side", and "face" mean the side or toward the side of the photographic element carrying the biaxially oriented polyolefin sheet. When referring to the embodiment comprising a biaxially oriented polyolefin sheet laminated to a transparent polymer support, the terms "bottom", "lower side", and "back" mean the side or toward the side opposite of the photographic element carrying the biaxially oriented polyolefin sheet. For the elements that do not have a laminated base, the terms "top", "upper", and "emulsion side" mean the side or toward the side carrying the emulsion layer. The

translucent sheets of the not laminated bases may be dupli-  
5 cated and for such dupli-  
cated elements "top", "upper", or  
"face side" is the side from which exposure takes place. The  
term as used herein, "transparent" means the ability to pass  
radiation without significant deviation or absorption. For  
this invention, "transparent" material is defined as a material  
that has a spectral transmission greater than 90%. The term  
as used herein, "translucent" is defined as a material that has  
a spectral transmission between 15% and 85%. The term as  
used herein, "reflective" is defined as a material that has a  
spectral transmission less than 15%. For a photographic  
element, spectral transmission is the ratio of the transmitted  
power to the incident power and is expressed as a percentage  
as follows:  $T_{RGB}=10^{-D}*100$  where D is the average of the  
10 red, green, and blue Status A transmission density response  
15 measured by an X-Rite model 310 (or comparable) photographic  
transmission densitometer. The term as used herein,  
"dupli-  
cated" means light sensitive silver halide coating on  
the top side and the bottom side of the imaging support.

20 It has been found that when photographic dyes are developed on a base that contains significant amounts of white pigments such as  $TiO_2$ , the dye hue angle of photographic dyes can change compared to the same dyes developed on a transparent base. Commonly used white pigments such as  $TiO_2$  corrupt the optical properties of the base to change the natural or inherent hue angle of photographic dyes. The observed change in dye hue between a transparent support and a support containing white pigments can be significant. Depending on the amount of white pigments used in a support, the dye hue change has been measured to be as much as 10 degrees. A 10-degree change in dye hue is undesirable, as the dye hue moves into a region that is not perceptually preferred. For example, a yellow dye hue angle of 98 degrees translates into a "green yellow" and is perceptually preferred over a yellow dye hue angle of 92 degrees which translates into a "red yellow". Further, the "green yellow" will attract more attention to the display material and, thus, be more effective than a "red yellow" at attracting the attention of the viewing public.

25 For the display materials of this invention, some level of light diffusion is needed so that the display light source is not apparent to the observer. Prior art display materials use white pigments coated in the emulsions bottom layers or incorporated into the base materials to diffuse light. In order 30 to provide the necessary amount of display light diffusion and maintain dye hue, it is desirable to remove the white pigments from imaging element. This has been accomplished without the loss of diffusion properties by the incorporation of several air/polymer interfaces in the display base material. The use of microvoided polyolefins and 35 polyester, in which air void sizes and void distribution can vary depending on the desired light transmission level, can 40 efficiently disuse the light and maintain the dye hue angle of the photographic dyes.

45 The invention has three described embodiments of translucent base materials: (1) microvoided biaxially oriented polyolefin sheet laminated to a transparent polymer base, (2) an integral composite biaxially oriented multilayer polyolefin sheet, and (3) an integral composite oriented multilayer 50 polyester sheet. These base materials are then coated either on the top side or both the top and bottom sides (dupli-  
cated) with light sensitive silver halide emulsion and processed after exposure using typical photographic wet chemistry.

55 Spectral transmission is the amount of light energy that is transmitted through a material. For a photographic element, spectral transmission the ratio of the transmitted power to the incident power and is expressed as a percentage as

follows:  $T_{RGB}=10^{-D}*100$  where D is the average of the red, green, and blue Status A transmission density response measured by an X-Rite model 310 (or comparable) photographic transmission densitometer. The higher the transmission, the less opaque the material. For a transmission display material with an incorporated diffuser, the quality of the image is related to the amount of light reflected from the image to the observer's eye. A display image with a low amount of spectral transmission does not allow sufficient illumination of the image causing a perceptual loss in image quality. The preferred spectral transmission of the translucent sheet of this invention is between 15% and 85%. A translucent polymer sheet with a spectral transmission greater than 90% does not sufficiently diffuse the lighting elements of the illuminating light source and, as a result, significantly reduces the commercial value of the image. A spectral transmission of less than 15% is difficult to obtain by the use of polymer voids.

The most preferred spectral transmission of the translucent polymer sheet of this invention is between 40% and 85% because this range of spectral transmission allows the illuminating light source to properly illuminate the image. Spectral transmission between 40% and 85% are typical of prior art transmission materials and perform well with existing transmission frames.

The translucent polymer base of this invention may also have an imaging forming layer applied to the top and bottom sides of the base. This duplitzed imaging forming layer allows for an increase in dye density, while still maintaining a 50 second developer time. Prior art transmission display materials typically have a high silver halide emulsion coverage on the top side to obtain the required dye density for a high quality transmission display image. This high emulsion coverage typically required a 110 second developer time. A 50 second developer time for the invention significantly improves the efficiency of the commercial development labs.

For the photographic element of this invention, after exposure and development the preferred change in hue angle is five degrees or less from the hue angle of the same dye coated, exposed, and developed on a substantially transparent base. Dye hue angle describes the color shade of the yellow, magenta, and cyan dyes used in the photographic element. Dye hue is important, as each dye has a perceptually preferred dye hue. Significant deviation from the perceptually preferred yellow, magenta, or cyan dye hue angle can result in a loss in perceived image quality for the transmission display. A hue angle change of greater than 6 degrees is undesirable, as it can reduce the effectiveness of the dye by moving the dye hue away from the intended angle. For example, a yellow dye with a hue angle of 98 degrees (green yellow) is perceptually preferred over a yellow dye with a hue angle of 92 degrees (red yellow).

Since the display materials of this invention are high in quality and have an improved dye hue angle compared to reflective photographic images, the display materials of this invention also have many consumer advantages. Home viewing of the display materials of this invention is possible with the use of a display apparatus that holds the display material and illuminates the display materials with an illumination light source. The display materials offer the consumer improved hue angles, sharp images, flat images, and an image that is high in gloss. Since the display materials are illuminated, the display materials can be viewed regardless of the ambient lighting conditions.

For the embodiment (1) of the invention comprising a biaxially oriented polyolefin sheet laminated to a transparent

polymer sheet, microvoided composite biaxially oriented polyolefin sheets are preferred because the voids provide opacity without the use of  $TiO_2$ . Microvoided composite oriented sheets are conveniently manufactured by coextrusion of the core and surface layers, followed by biaxial orientation, whereby voids are formed around void-initiating material contained in the core layer. Such composite sheets are disclosed in, for example, U.S. Pat. Nos. 4,377,616; 4,758,462; and 4,632,869. As the base of the laminate is transparent, the light transmission of the laminate of embodiment (1) is substantially the same as the light transmission of the voided biaxially oriented sheet laminated to the transparent sheet.

The core of the preferred composite sheet should be from 15 to 95% of the total thickness of the sheet, preferably from 30 to 85% of the total thickness. The nonvoided skin(s) should thus be from 5 to 85% of the sheet, preferably from 15 to 70% of the thickness.

The density (specific gravity) of the composite sheet, expressed in terms of "percent of solid density" is calculated as follows:

$$\frac{\text{Composite Sheet Density}}{\text{Polymer Density}} \times 100 = \% \text{ of Solid Density}$$

25

should be between 45% and 100%, preferably between 67% and 100%. As the percent solid density becomes less than 67%, the composite sheet becomes less manufacturable due to a drop in tensile strength and it becomes more susceptible to physical damage.

The total thickness of the composite sheet can range from 12 to 100 micrometers, preferably from 20 to 70  $\mu m$ . Below 20  $\mu m$ , the microvoided sheets may not be thick enough to minimize any inherent nonplanarity in the support and would be more difficult to manufacture. At thickness higher than 70  $\mu m$ , little improvement in either surface smoothness or mechanical properties are seen, and so there is little justification for the further increase in cost for extra materials.

"Void" is used herein to mean devoid of added solid and liquid matter, although it is likely the "voids" contain gas. The void-initiating particles which remain in the finished packaging sheet core should be from 0.1 to 10  $\mu m$  in diameter, preferably round in shape, to produce voids of the desired shape and size. The size of the void is also dependent on the degree of orientation in the machine and transverse directions. Ideally, the void would assume a shape which is defined by two opposed and edge contacting concave disks. In other words, the voids tend to have a lens-like or biconvex shape. The voids are oriented so that the two major dimensions are aligned with the machine and transverse directions of the sheet. The Z-direction axis is a minor dimension and is roughly the size of the cross diameter of the voiding particle. The voids generally tend to be closed cells and, thus, there is virtually no path open from one side of the voided-core to the other side through which gas or liquid can traverse.

The void-initiating material may be selected from a variety of materials, and should be present in an amount of about 5-50% by weight based on the weight of the core matrix polymer. Preferably, the void-initiating material comprises a polymeric material. When a polymeric material is used, it may be a polymer that can be melt-mixed with the polymer from which the core matrix is made and be able to form dispersed spherical particles as the suspension is cooled down. Examples of this would include nylon dis-

persed in polypropylene, polybutylene terephthalate in polypropylene, or polypropylene dispersed in polyethylene terephthalate. If the polymer is preshaped and blended into the matrix polymer, the important characteristic is the size and shape of the particles. Spheres are preferred and they can be hollow or solid. These spheres may be made from cross-linked polymers which are members selected from the group consisting of an alkenyl aromatic compound having the general formula Ar—C(R)=CH<sub>2</sub>, wherein Ar represents an aromatic hydrocarbon radical, or an aromatic halohydrocarbon radical of the benzene series and R is hydrogen or the methyl radical; acrylate-type monomers include monomers of the formula CH<sub>2</sub>=C(R')—C(O)(OR) wherein R is selected from the group consisting of hydrogen and an alkyl radical containing from about 1 to 12 carbon atoms and R' is selected from the group consisting of hydrogen and methyl; copolymers of vinyl chloride and vinylidene chloride, acrylonitrile and vinyl chloride, vinyl bromide, vinyl esters having formula CH<sub>2</sub>=CH(O)COR, wherein R is an alkyl radical containing from 2 to 18 carbon atoms; acrylic acid, methacrylic acid, itaconic acid, citraconic acid, maleic acid, fumaric acid, oleic acid, vinylbenzoic acid; the synthetic polyester resins which are prepared by reacting terephthalic acid and dialkyl terephthalates or ester-forming derivatives thereof, with a glycol of the series HO(CH<sub>2</sub>)<sub>n</sub>OH wherein n is a whole number within the range of 2-10 and having reactive olefinic linkages within the polymer molecule, the above described polyesters which include copolymerized therein up to 20 percent by weight of a second acid or ester thereof having reactive olefinic unsaturation and mixtures thereof, and a cross-linking agent selected from the group consisting of divinylbenzene, diethylene glycol dimethacrylate, diallyl fumarate, diallyl phthalate and mixtures thereof.

Examples of typical monomers for making the cross-linked polymer include styrene, butyl acrylate, acrylamide, acrylonitrile, methyl methacrylate, ethylene glycol dimethacrylate, vinyl pyridine, vinyl acetate, methyl acrylate, vinylbenzyl chloride, vinylidene chloride, acrylic acid, divinylbenzene, acrylamidomethylpropane sulfonic acid, vinyl toluene, etc. Preferably, the cross-linked polymer is polystyrene or poly(methyl methacrylate). Most preferably, it is polystyrene and the cross-linking agent is divinylbenzene.

Processes well known in the art yield nonuniformly sized particles, characterized by broad particle size distributions. The resulting beads can be classified by screening the beads spanning the range of the original distribution of sizes. Other processes, such as suspension polymerization and limited coalescence, directly yield very uniformly sized particles.

The void-initiating materials may be coated with agents to facilitate voiding. Suitable agents or lubricants include colloidal silica, colloidal alumina, and metal oxides such as tin oxide and aluminum oxide. The preferred agents are colloidal silica and alumina, most preferably, silica. The cross-linked polymer having a coating of an agent may be prepared by procedures well known in the art. For example, conventional suspension polymerization processes wherein the agent is added to the suspension is preferred. As the agent, colloidal silica is preferred.

The void-initiating particles can also be inorganic spheres, including solid or hollow glass spheres, metal or ceramic beads or inorganic particles such as clay, talc, barium sulfate, and calcium carbonate. The important thing is that the material does not chemically react with the core matrix polymer to cause one or more of the following problems: (a) alteration of the crystallization kinetics of the

matrix polymer, making it difficult to orient, (b) destruction of the core matrix polymer, (c) destruction of the void-initiating particles, (d) adhesion of the void-initiating particles to the matrix polymer, or (e) generation of undesirable reaction products, such as toxic or high color moieties. The void-initiating material should not be photographically active or degrade the performance of the photographic element in which the biaxially oriented polyolefin film is utilized.

For the biaxially oriented sheets on the top side toward the emulsion, suitable classes of thermoplastic polymers for the biaxially oriented sheet and the core matrix-polymer of the preferred composite sheet comprise polyolefins. Suitable polyolefins include polypropylene, polyethylene, polymethylpentene, polystyrene, polybutylene, and mixtures thereof. Polyolefin copolymers, including copolymers of propylene and ethylene such as hexene, butene, and octene, are also useful. Polypropylene is preferred, as it is low in cost and has desirable strength properties.

The nonvoided skin layers of the composite sheet can be made of the same polymeric materials as listed above for the core matrix. The composite sheet can be made with skin(s) of the same polymeric material as the core matrix, or it can be made with skin(s) of different polymeric composition than the core matrix.

The total thickness of the top most skin layer or exposed surface layer should be between 0.20  $\mu\text{m}$  and 1.5  $\mu\text{m}$ , preferably between 0.5 and 1.0  $\mu\text{m}$ . Below 0.5  $\mu\text{m}$  any inherent nonplanarity in the coextruded skin layer may result in unacceptable color variation. At skin thickness greater than 1.0  $\mu\text{m}$ , there is a reduction in the photographic optical properties such as image resolution. At thickness greater than 1.0  $\mu\text{m}$  there is also a greater material volume to filter for contamination such as clumps, poor color pigment dispersion, or contamination. Low density polyethylene with a density of 0.88 to 0.94 g/cc is the preferred material for the top skin because current emulsion formulation adhere well to low density polyethylene compared to other materials such as polypropylene and high density polyethylene.

Addenda may be added to the topmost skin layer to change the color of the imaging element. For photographic use, a white base with a slight bluish tinge is preferred. The addition of the slight bluish tinge may be accomplished by any process which is known in the art, including the machine blending of color concentrate prior to extrusion and the melt extrusion of blue colorants that have been pre-blended at the desired blend ratio. Colored pigments that can resist extrusion temperatures greater than 320° C. are preferred, as temperatures greater than 320° C. are necessary for coextrusion of the skin layer. Blue colorants used in this invention may be any blue colorant that does not have an adverse impact on the imaging element. Preferred blue colorants include Phthalocyanine blue pigments, Cromophthal blue pigments, Irgazin blue pigments, Irgalite organic blue pigments, and pigment Blue 60.

It has been found that a very thin coating (0.2 to 1.5  $\mu\text{m}$ ) on the surface immediately below the emulsion layer can be made by coextrusion and subsequent stretching in the width and length direction. It has been found that this layer is, by nature, extremely accurate in thickness and can be used to provide all the color corrections which are usually distributed throughout the thickness of the sheet between the emulsion and the paper base. This topmost layer is so efficient that the total colorants needed to provide a correction are less than one-half the amount needed if the colorants are dispersed throughout thickness. Colorants are often the cause of spot defects due to clumps and poor dispersions.

Spot defects, which decrease the commercial value of images, are improved with this invention because less colorant is used and high quality filtration to clean up the colored layer is much more feasible since the total volume of polymer with colorant is only typically 2 to 10 percent of the total polymer between the base paper and the photosensitive layer.

Addenda may be added to the biaxially oriented sheet of this invention so that when the biaxially oriented sheet is viewed by the intended audience, the imaging element emits light in the visible spectrum when exposed to ultraviolet radiation. Emission of light in the visible spectrum allows for the support to have a desired background color in the presence of ultraviolet energy. This is particularly useful when images are backlit with a light source that contains ultraviolet energy and may be used to optimize image quality for transmission display applications.

Addenda known in the art to emit visible light in the blue spectrum are preferred. Consumers generally prefer a slight blue tint to white defined as a negative  $b^*$  compared to a white white defined as a  $b^*$  within one  $b^*$  unit of zero.  $b^*$  is the measure of yellow/blue in CIE space. A positive  $b^*$  indicates yellow, while a negative  $b^*$  indicates blue. The addition of addenda that emits in the blue spectrum allows for tinting the support without the addition of colorants which would decrease the whiteness of the image. The preferred emission is between 1 and 5 delta  $b^*$  units. Delta  $b^*$  is defined as the  $b^*$  difference measured when a sample is an illuminated ultraviolet light source and a light source without any significant ultraviolet energy. Delta  $b^*$  is the preferred measure to determine the net effect of adding an optical brightener to the top biaxially oriented sheet of this invention. Emissions less than 1  $b^*$  unit cannot be noticed by most customers; therefore, is it not cost effective to add small amounts of optical brightener to the biaxially oriented sheet. An emission greater than 5  $b^*$  units would interfere with the color balance of the prints making the whites appear too blue for most consumers.

The preferred addenda of this invention is an optical brightener. An optical brightener is a substantially colorless, fluorescent, organic compound that absorbs ultraviolet light and emits it as visible blue light. Examples include, but are not limited to, derivatives of 4,4'-diaminostilbene-2,2'-disulfonic acid, coumarin derivatives such as 4-methyl-7-diethylaminocoumarin, 1-4-Bis(O-Cyanostyryl)Benzol, and 2-Amino-4-Methyl Phenol. An unexpected desirable feature of this invention is the efficient use of optical brightener. Because the ultraviolet source for a transmission display material is on the opposite side of the image, the ultraviolet light intensity is not reduced by ultraviolet filters common to imaging layers. The result is that less optical brightener is required to achieve the desired background color.

The optical brightener may be added to any layer in the multilayer coextruded biaxially oriented polyolefin sheet. The preferred location is adjacent to or in the exposed surface layer of said sheet. This allows for the efficient concentration of optical brightener which results in less optical brightener being used when compared to traditional photographic supports. When the desired weight % loading of the optical brightener begins to approach the concentration at which the optical brightener migrates to the surface of the support forming crystals in the imaging layer, the addition of optical brightener into the layer adjacent to the exposed layer is preferred. When optical brightener migration is a concern as with light sensitive silver halide imaging systems, the preferred exposed layer comprised polyethylene. In this case, the migration from the layer adjacent to the

exposed layer is significantly reduced because the surface layer acts as a barrier layer allowing for much higher optical brightener levels to be used to optimize image quality. Locating the optical brightener in the layer adjacent to the exposed layer allows for a less expensive optical brightener to be used as the exposed layer, which is substantially free of optical brightener, and prevents significant migration of the optical brightener. Another preferred method to reduce unwanted optical brightener migration is to use polypropylene for the layer adjacent to the exposed surface. Since optical brightener is more soluble in polypropylene than polyethylene, the optical brightener is less likely to migrate from polypropylene.

A biaxially oriented sheet of this invention which has a microvoided core is preferred. The microvoided core adds opacity and whiteness to the imaging support further improving imaging quality. Further, the voided core is an excellent diffuser of light and has substantially less light scatter than white pigments such as  $TiO_2$ . Less light scatter improves the quality of the transmitted image. Combining the image quality advantages of a microvoided core with a material, which absorbs ultraviolet energy and emits light in the visible spectrum, allows for the unique optimization of image quality as the image support can have a tint when exposed to ultraviolet energy, yet retain excellent whiteness when the image is viewed using lighting that does not contain significant amounts of ultraviolet energy such as indoor lighting. The preferred number of voids in the vertical direction at substantially every point is greater than six. The number of voids in the vertical direction is the number of polymer/gas interfaces present in the voided layer. The voided layer functions as an opaque layer because of the index of refraction changes between polymer/gas interfaces. Greater than 6 voids is preferred because at 4 voids or less, little improvement in the opacity of the film is observed and, thus, does not justify the added expense to void the biaxially oriented sheet of this invention. Between 6 and 30 voids in the vertical direction is most preferred because at 35 voids or greater the voided core can be easily stressed fractured resulting in undesirable fracture lines in the image area which reduce the commercial value of the transmission display material.

The coextrusion, quenching, orienting, and heat setting of these composite sheets may be effected by any process which is known in the art for producing oriented sheet, such as by a flat sheet process or a bubble or tubular process. The flat sheet process involves extruding the blend through a slit die and rapidly quenching the extruded web upon a chilled casting drum so that the core matrix polymer component of the sheet and the skin component(s) are quenched below their glass solidification temperature. The quenched sheet is then biaxially oriented by stretching in mutually perpendicular directions at a temperature above the glass transition temperature, below the melting temperature of the matrix polymers. The sheet may be stretched in one direction and then in a second direction or may be simultaneously stretched in both directions. A stretching ratio, defined as the final length divided by the original length for sum of the machine and cross directions, of at least 10 to 1 is preferred. After the sheet has been stretched, it is heat set by heating to a temperature sufficient to crystallize or anneal the polymers, while restraining to some degree the sheet against retraction in both directions of stretching.

The composite sheet, while described as having preferably at least three layers of a core and a skin layer on each side, may also be provided with additional layers that may serve to change the properties of the biaxially oriented sheet.

Biaxially oriented sheets could be formed with surface layers that would provide an improved adhesion, or look to the support and photographic element. The biaxially oriented extrusion could be carried out with as many as 10 layers if desired to achieve some particular desired property.

These composite sheets may be coated or treated after the coextrusion and orienting process or between casting and full orientation with any number of coatings, which may be used to improve the properties of the sheets including printability to provide a vapor barrier, to make them heat sealable, or to improve the adhesion to the support or to the photosensitive layers. Examples of this would be acrylic coatings for printability and coating polyvinylidene chloride for heat seal properties. Further examples include flame, plasma, or corona discharge treatment to improve printability or adhesion.

By having at least one nonvoided skin on the microvoided core, the tensile strength of the sheet is increased and makes it more manufacturable. It allows the sheets to be made at wider widths and higher draw ratios than when sheets are made with all layers voided. Coextruding the layers further simplifies the manufacturing process.

The structure of a preferred biaxially oriented polyolefin sheet where the exposed surface layer is adjacent to the imaging layer is as follows:

---

Polyethylene skin with blue pigments (top layer)  
 Polypropylene with optical brightener  
 Polypropylene microvoided layer  
 Polypropylene bottom skin layer

---

The support to which the biaxially oriented polyolefin sheets are laminated for the laminated support of the photosensitive silver halide layer may be any material with the desired transmission and stiffness properties. Photographic elements of the invention can be prepared on any suitable transparent photographic quality support including materials such as polystyrene, synthetic high molecular weight sheet materials such as polyalkyl acrylates or methacrylates, polystyrene, polyamides such as nylon, sheets of semisynthetic high molecular weight materials such as cellulose nitrate, cellulose acetate butyrate, and the like; homo and copolymers of vinyl chloride, poly(vinylacetal), polycarbonates, homo and copolymers of olefins such as polyethylene and polypropylene, and the like.

Polyester sheets are particularly advantageous because they provide excellent strength, dimensional stability and are transparent. Such polyester sheets are well known, widely used in display materials, and typically prepared from high molecular weight polyesters prepared by condensing a dihydric alcohol with a dibasic saturated fatty acid or derivative thereof.

Suitable dihydric alcohols for use in preparing such polyesters are well known in the art and include any glycol wherein the hydroxyl groups are on the terminal carbon atom and contain from 2 to 12 carbon atoms such as, for example, ethylene glycol, propylene glycol, trimethylene glycol, hexamethylene glycol, decamethylene glycol, dodecamethylene glycol, 1,4-cyclohexane, dimethanol, and the like.

Suitable dibasic acids useful for the preparation of polyesters include those containing from 2 to 16 carbon atoms such as adipic acid, sebatic acid, isophthalic acid, terephthalic acid, and the like. Alkyl esters of acids such as those listed above can also be employed. Other alcohols and acids, as well as polyesters prepared therefrom and the preparation of

the polyesters, are described in U.S. Pat. Nos. 2,720,503 and 2,901,466. Polyethylene terephthalate is preferred.

Polyester support stiffness can range from about 15 millinewtons to 100 millinewtons. The preferred stiffness is between 20 and 100 millinewtons. Polyester stiffness less than 15 millinewtons does not provide the required stiffness for display materials in that they will be difficult to handle and do not lay flat for optimum viewing. Polyester stiffness greater than 100 millinewtons begins to exceed the stiffness limit for processing equipment and has no performance benefit for the display materials.

Generally polyester supports are prepared by melt extruding the polyester through a slit die, quenching to the amorphous state, orienting by machine and cross direction stretching, and heat setting under dimensional restraint. The polyester film can also be subjected to a heat relaxation treatment to improve dimensional stability and surface smoothness.

The polyester film will typically contain an undercoat 20 subbing or primer layer on both sides of the polyester film. Subbing layers used to promote adhesion of coating compositions to the support are well known in the art, and any such material can be employed. Some useful compositions for this purpose include interpolymers of vinylidene chloride 25 such as vinylidene chloride/methyl acrylate/itaconic acid terpolymers or vinylidene chloride/acrylonitrile/acrylic acid terpolymers, and the like. These and other suitable compositions are described, for example, in U.S. Pat. Nos. 2,627, 088; 2,698,240; 2,943,937; 3,143,421; 3,201,249; 3,271, 178; 3,443,950; and 3,501,301. The polymeric subbing layer 30 is usually overcoated with a second subbing layer comprised of gelatin, typically referred to as gel sub.

A transparent polymer base free of  $TiO_2$  is preferred because the  $TiO_2$  in the transparent polymer gives the 35 reflective display materials an undesirable opalescence appearance and changes hue. The  $TiO_2$  pigmented transparent polymer also is expensive because the  $TiO_2$  must be dispersed into the entire thickness, typically from 100 to 180  $\mu m$ . The  $TiO_2$  also gives the transparent polymer support a 40 slight yellow tint which is undesirable for a photographic display material. For use as a photographic reflective display material, a transparent polymer support containing  $TiO_2$  must also be tinted blue to offset the yellow tint of the polyester, causing a loss in desired whiteness and adding cost to the display material. Concentration of the white pigment in the polyolefin layer allows for efficient use of the white pigment which improves image quality and reduces the cost of the imaging support.

When using a polyester base sheet, it is preferable to 50 extrusion laminate the microvoided composite sheets to the polyester sheet using a polyolefin resin. Extrusion laminating is carried out by bringing together the biaxially oriented sheets of the invention and the polyester base with application of a melt extruded adhesive between the polyester sheets and the biaxially oriented polyolefin sheets, followed by their being pressed in a nip such as between two rollers. The melt extruded adhesive may be applied to either the 55 biaxially oriented sheets or the base polyester sheet prior to their being brought into the nip. In a preferred form the adhesive is applied into the nip simultaneously with the biaxially oriented sheets and the base polyester sheet. The adhesive used to adhere the biaxially oriented polyolefin sheet to the polyester base may be any suitable material that does not have a harmful effect upon the photographic element. A preferred material is metallocene catalyzed ethylene plastomers that are melt extruded into the nip between the polyester sheet and the biaxially oriented sheet. Metal-

## 13

locene catalyzed ethylene plastomers are preferred because they are easily melt extruded, adhere well to biaxially oriented polyolefin sheets of this invention, and adhere well to gelatin subbed polyester support of this invention.

The structure of a preferred display support where the imaging layers are applied to the biaxially oriented polyolefin sheet is as follows:

---

Biaxially oriented polyolefin sheet  
Metallocene catalyzed ethylene plastomer  
Polyester base

---

Another embodiment of a translucent polymer base for the photographic element of this invention is a multilayer voided polyester base sheet. The polyester should have a glass transition temperature between about 50° C. and about 150° C., preferably about 60–100° C., should be orientable, and have an IV of at least 0.50, preferably 0.6 to 0.9. Suitable polyesters include those produced from aromatic, aliphatic or cyclo-aliphatic dicarboxylic acids of 4–20 carbon atoms and aliphatic or alicyclic glycols having from 2–24 carbon atoms. Examples of suitable dicarboxylic acids include terephthalic, isophthalic, phthalic, naphthalene dicarboxylic acid, succinic, glutaric, adipic, azelaic, sebacic, fumaric, maleic, itaconic, 1,4-cyclohexane-dicarboxylic, sodiosulfoiso-phthalic, and mixtures thereof. Examples of suitable glycols include ethylene glycol, propylene glycol, butanediol, pentanediol, hexanediol, 1,4-cyclohexane-dimethanol, diethylene glycol, other polyethylene glycols, and mixtures thereof. Such polyesters are well known in the art and may be produced by well-known techniques, e.g., those described in U.S. Pat. Nos. 2,465,319 and 2,901,466. Preferred continuous matrix polymers are those having repeat units from terephthalic acid or naphthalene dicarboxylic acid and at least one glycol selected from ethylene glycol, 1,4-butanediol and 1,4-cyclohexanedimethanol. Poly(ethylene terephthalate), which may be modified by small amounts of other monomers, is especially preferred. Polypropylene is also useful. Other suitable polyesters include liquid crystal copolymers formed by the inclusion of a suitable amount of a co-acid component such as stilbene dicarboxylic acid. Examples of such liquid crystal copolymers are those disclosed in U.S. Pat. Nos. 4,420,607; 4,459,402; and 4,468,510.

Suitable cross-linked polymers for the microbeads, for voiding polyester sheet, are polymerizable organic materials which are members selected from the group consisting of an alkenyl aromatic compound having the general formula



wherein Ar represents an aromatic hydrocarbon radical, or an aromatic halohydrocarbon radical of the benzene series and R is hydrogen or the methyl radical; acrylate-type monomers including monomers of the formula



wherein R is selected from the group consisting of hydrogen and an alkyl radical containing from about 1 to 12 carbon atoms and R' is selected from the group consisting of

## 14

hydrogen and methyl; copolymers of vinyl chloride and vinylidene chloride, acrylonitrile and vinyl chloride, vinyl bromide, vinyl esters having the formula



wherein R is an alkyl radical containing from 2 to 18 carbon atoms; acrylic acid, methacrylic acid, itaconic acid, citraconic acid, maleic acid, fumaric acid, oleic acid, vinylbenzoic acid; the synthetic polyester resins which are prepared by reacting terephthalic acid and dialkyl terephthalates or ester-forming derivatives thereof, with a glycol of the series 10  $\text{HO}(\text{CH}_2)_n\text{OH}$ , wherein n is a whole number within the range of 2–10 and having reactive olefinic linkages within the polymer molecule, the hereinabove described polyesters which include copolymerized therein up to 20 percent by weight of a second acid or ester thereof having reactive olefinic unsaturation and mixtures thereof, and a cross-linking agent selected from the group consisting of divinylbenzene, diethylene glycol dimethacrylate, oiallyl fumarate, diallyl phthalate and mixtures thereof.

Examples of typical monomers for making the cross-linked polymer include styrene, butyl acrylate, acrylamide, 25 acrylonitrile, methyl methacrylate, ethylene glycol dimethacrylate, vinyl pyridine, vinyl acetate, methyl acrylate, vinylbenzyl chloride, vinylidene chloride, acrylic acid, divinylbenzene, arylamidomethyl-propane sulfonic acid, vinyl toluene, etc. Preferably, the cross-linked polymer 30 is polystyrene or poly(methyl methacrylate). Most preferably, it is polystyrene and the cross-linking agent is divinylbenzene.

Processes well known in the art yield nonuniformly sized particles, characterized by broad particle size distributions. 35 The resulting beads can be classified by screening to produce beads spanning the range of the original distribution of sizes. Other processes such as suspension polymerization and limited coalescence directly yield very uniformly sized particles. Suitable slip agents or lubricants include colloidal 40 silica, colloidal alumina, and metal oxides such as tin oxide and aluminum oxide. The preferred slip agents are colloidal silica and alumina, most preferably, silica. The cross-linked polymer having a coating of slip agent may be prepared by procedures well known in the art. For example, conventional 45 suspension polymerization processes wherein the slip agent, colloidal silica is added to the suspension is preferred. As the slip agent, colloidal silica is preferred.

It is preferred to use the “limited coalescence” technique 50 for producing the coated, cross-linked polymer microbeads. This process is described in detail in U.S. Pat. No. 3,615, 55 972. Preparation of the coated microbeads for use in the present invention does not utilize a blowing agent as described in this patent, however. The following general procedure may be utilized in a limited coalescence technique:

1. The polymerizable liquid is dispersed within an aqueous nonsolvent liquid medium to form a dispersion of droplets having sizes not larger than the size desired for the polymer globules, whereupon
2. The dispersion is allowed to rest and to reside with only mild or no agitation for a time during which a limited coalescence of the dispersed droplets takes place with the formation of a lesser number of larger droplets, such coalescence being limited due to the composition of the suspending medium, the size of the dispersed droplets thereby becoming remarkably uniform and of a desired magnitude, and

3. The uniform droplet dispersion is then stabilized by addition of thickening agents to the aqueous suspending medium, whereby the uniform-sized dispersed droplets are further protected against coalescence and are also retarded from concentrating in the dispersion due to difference in density of the disperse phase and continuous phase, and
4. The polymerizable liquid or oil phase in such stabilized dispersion is subjected to polymerization conditions and polymerized, whereby globules of polymer are obtained having spheroidal shape and remarkably uniform and desired size, which size is predetermined principally by the composition of the initial aqueous liquid suspending medium.

The diameter of the droplets of polymerizable liquid, and hence the diameter of the beads of polymer, can be varied predictably, by deliberate variation of the composition of the aqueous liquid dispersion, within the range of from about one-half of a micrometer or less to about 0.5 centimeter. For any specific operation, the range of diameters of the droplets of liquid, and hence of polymer beads, has a factor in the order of three or less as contrasted to factors of 10 or more for diameters of droplets and beads prepared by usual suspension polymerization methods employing critical agitation procedures. Since the bead size, e.g., diameter, in the present method is determined principally by the composition of the aqueous dispersion, the mechanical conditions, such as the degree of agitation, the size and design of the apparatus used, and the scale of operation, are not highly critical. Furthermore, by employing the same composition, the operations can be repeated, or the scale of operations can be changed, and substantially the same results can be obtained.

The present method is carried out by dispersing one part by volume of a polymerizable liquid into at least 0.5, preferably from 0.5 to about 10 or more, parts by volume of a nonsolvent aqueous medium comprising water and at least the first of the following ingredients:

1. A water-dispersible, water-insoluble solid colloid, the particles of which, in aqueous dispersion, have dimensions in the order of from about 0.008 to about 50  $\mu\text{m}$ , which particles tend to gather at the liquid-liquid interface or are caused to do so by the presence of
2. A water-soluble "promoter" that affects the "hydrophilic-hydrophobic balance" of the solid colloid particles; and/or
3. An electrolyte; and/or
4. Colloid-active modifiers such as peptizing agents, surface-active agents and the like; and usually
5. A water-soluble, monomer-insoluble inhibitor of polymerization.

The water-dispersible, water-insoluble solid colloids can be inorganic materials such as metal salts or hydroxides or clays, or can be organic materials such as raw starches, sulfonated cross-linked organic high polymers, resinous polymers, and the like.

The solid colloidal material must be insoluble, but dispersible in water and both insoluble and nondispersible in, but wettable by, the polymerizable liquid. The solid colloids must be much more hydrophilic than oleophilic so as to remain dispersed wholly within the aqueous liquid. The solid colloids employed for limited coalescence are ones having particles that, in the aqueous liquid, retain a relatively rigid and discrete shape and size within the limits stated. The particles may be greatly swollen and extensively hydrated, provided that the swollen particle retains a definite

shape, in which case the effective size is approximately that of the swollen particle. The particles can be essentially single molecules, as in the case of extremely high molecular weight cross-linked resins, or can be aggregates of many molecules. Materials that disperse in water to form true or colloidal solutions in which the particles have a size below the range stated or in which the particles are so diffuse as to lack a discernible shape and dimension are not suitable as stabilizers for limited coalescence. The amount of solid colloid that is employed is usually such as corresponds to from about 0.01 to about 10 or more grams per 100 cubic centimeters of the polymerizable liquid.

In order to function as a stabilizer for the limited coalescence of the polymerizable liquid droplets, it is essential that the solid colloid must tend to collect with the aqueous liquid at the liquid-liquid interface, i.e., on the surface of the oil droplets. (The term "oil" is occasionally used herein as generic to liquids that are insoluble in water.) In many instances, it is desirable to add a "promoter" material to the aqueous composition to drive the particles of the solid colloid to the liquid-liquid interface. This phenomenon is well known in the emulsion art, and is here applied to solid colloidal particles, as an expanded of adjusting the "hydrophilic-hydrophobic balance."

Usually, the promoters are organic materials that have an affinity for the solid colloid and also for the oil droplets and that are capable of making the solid colloid more oleophilic. The affinity for the oil surface is usually due to some organic portion of the promoter molecule, while affinity for the solid colloid is usually due to opposite electrical charges. For example, positively charged complex metal salts or hydroxides, such as aluminum hydroxide, can be promoted by the presence of negatively charged organic promoters such as water-soluble sulfonated polystyrenes, alignates, and carboxymethylcellulose. Negatively charged colloids, such as Bentonite, are promoted by positively charged promoters such as tetramethyl ammonium hydroxide or chloride or water-soluble complex resinous amine condensation products, such as the water-soluble condensation products of diethanolamine and adipic acid, the water-soluble condensation products of ethylene oxide, urea and formaldehyde, and polyethylenimine. Amphoteric materials such as proteinaceous materials like gelatin, glue, casein, albumin, glutin and the like are effective promoters for a wide variety of colloidal solids. Nonionic materials like methoxy-cellulose are also effective in some instances. Usually, the promoter need be used only to the extent of a few parts per million of aqueous medium, although larger proportions can often be tolerated. In some instances, ionic materials normally classed as emulsifiers, such as soaps, long chain sulfates and sulfonates and the long chain quaternary ammonium compounds, can also be used as promoters for the solid colloids, but care must be taken to avoid causing the formation of stable colloidal emulsions of the polymerizable liquid and the aqueous liquid medium.

An effect similar to that of organic promoters is often obtained with small amounts of electrolytes, e.g., water-soluble, ionizable alkalies, acids, and salts, particularly those having polyvalent ions. These are especially useful when the excessive hydrophilic or insufficient oleophilic characteristic of the colloid is attributable to excessive hydration of the colloid structure. For example, a suitably cross-linked sulfonated polymer of styrene is tremendously swollen and hydrated in water. Although the molecular structure contains benzene rings which should confer on the colloid some affinity for the oil phase in the dispersion, the great degree of hydration causes the colloidal particles to be enveloped in

a cloud of associated water. The addition of a soluble, ionizable polyvalent cationic compound, such as an aluminum or calcium salt, to the aqueous composition causes extensive shrinking of the swollen colloid with exudation of a part of the associated water and exposure of the organic portion of the colloid particle, thereby making the colloid more oleophilic.

The solid colloidal particles, whose hydrophilic-hydrophobic balance is such that the particles tend to gather in the aqueous phase at the oil-water interface, gather on the surface of the oil droplets and function as protective agents during limited coalescence.

Other agents that can be employed in an already known manner to effect modification of the colloidal properties of the aqueous composition are those materials known in the art as peptizing agents, flocculating and deflocculating agents, sensitizers, surface active agents, and the like.

It is sometimes desirable to add to the aqueous liquid a few parts per million of a water-soluble, oil-insoluble inhibitor of polymerization effective to prevent the polymerization of monomer molecules that might diffuse into the aqueous liquid or that might be absorbed by colloid micelles and that, if allowed to polymerize in the aqueous phase, would tend to make emulsion-type polymer dispersions instead of, or in addition to, the desired bead or pearl polymers.

The aqueous medium containing the water-dispersible solid colloid is then admixed with the liquid polymerizable material in such a way as to disperse the liquid polymerizable material as small droplets within the aqueous medium. This dispersion can be accomplished by any usual means, e.g., by mechanical stirrers or shakers, by pumping through jets, by impingement, or by other procedures causing subdivision of the polymerizable material into droplets in a continuous aqueous medium.

The degree of dispersion, e.g., by agitation is not critical except that the size of the dispersed liquid droplets must be no larger, and is preferably much smaller, than the stable droplet size expected and desired in the stable dispersion. When such condition has been attained, the resulting dispersion is allowed to rest with only mild, gentle movement, if any, and preferably without agitation. Under such quiescent conditions, the dispersed liquid phase undergoes a limited degree of coalescence.

"Limited coalescence" is a phenomenon wherein droplets of liquid dispersed in certain aqueous suspending media coalesce, with formation of a lesser number of larger droplets, until the growing droplets reach a certain critical and limiting size, whereupon coalescence substantially ceases. The resulting droplets of dispersed liquid, which can be as large as 0.3 and sometimes 0.5 centimeter in diameter, are quite stable as regards further coalescence and are remarkably uniform in size. If such a large droplet dispersion be vigorously agitated, the droplets are fragmented into smaller droplets. The fragmented droplets, upon quiescent standing, again coalesce to the same limited degree and form the same uniform-sized, large droplet, stable dispersion. Thus, a dispersion resulting from the limited coalescence comprises droplets of substantially uniform diameter that are stable in respect to further coalescence.

The principles underlying this phenomenon have now been adapted to cause the occurrence of limited coalescence in a deliberate and predictable manner in the preparation of dispersions of polymerizable liquids in the form of droplets of uniform and desired size.

In the phenomenon of limited coalescence, the small particles of solid colloid tend to collect with the aqueous liquid at the liquid-liquid interface, i.e., on the surface of the

oil droplets. It is thought that droplets which are substantially covered by such solid colloid are stable to coalescence, while droplets which are not so covered are not stable. In a given dispersion of a polymerizable liquid, the total surface area of the droplets is a function of the total volume of the liquid and the diameter of the droplets. Similarly, the total surface area barely coverable by the solid colloid, e.g., in a layer one particle thick, is a function of the amount of the colloid and the dimensions of the particles thereof. In the dispersion as initially prepared, e.g., by agitation, the total surface area of the polymerizable liquid droplets is greater than can be covered by the solid colloid. Under quiescent conditions, the unstable droplets begin to coalesce. The coalescence results in a decrease in the number of oil droplets and a decrease in the total surface area thereof up to a point at which the amount of colloidal solid is barely sufficient substantially to cover the total surface of the oil droplets, whereupon coalescence substantially ceases.

If the solid colloidal particles do not have nearly identical dimensions, the average effective dimension can be estimated by statistical methods. For example, the average effective diameter of spherical particles can be computed as the square root of the average of the squares of the actual diameters of the particles in a representative sample.

It is usually beneficial to treat the uniform droplet suspension prepared as described above to render the suspension stable against congregation of the oil droplets.

This further stabilization is accomplished by gently admixing with the uniform droplet dispersion an agent capable of greatly increasing the viscosity of the aqueous liquid. For this purpose, there may be used any water-soluble or water-dispersible thickening agent that is insoluble in the oil droplets and that does not remove the layer of solid colloidal particles covering the surface of the oil droplets at the oil-water interface. Examples of suitable thickening agents are sulfonated polystyrene (water-dispersible, thickening grade), hydrophilic clays such as Bentonite, digested starch, natural gums, carboxy-substituted cellulose ethers, and the like. Often the thickening agent is selected and employed in such quantities as to form a thixotropic gel in which are suspended the uniform-sized droplets of the oil. In other words, the thickened liquid generally should be non-Newtonian in its fluid behavior, i.e., of such a nature as to prevent rapid movement of the dispersed droplets within the aqueous liquid by the action of gravitational force due to the difference in density of the phases. The stress exerted on the surrounding medium by a suspended droplet is not sufficient to cause rapid movement of the droplet within such non-Newtonian media. Usually, the thickener agents are employed in such proportions relative to the aqueous liquid that the apparent viscosity of the thickened aqueous liquid is in the order of at least 500 centipoises (usually determined by means of a Brookfield viscosimeter using the No. 2 spindle at 30 rpm.). The thickening agent is preferably prepared as a separate concentrated aqueous composition that is then carefully blended with the oil droplet dispersion.

The resulting thickened dispersion is capable of being handled, e.g., passed through pipes, and can be subjected to polymerization conditions substantially without mechanical change in the size or shape of the dispersed oil droplets.

The resulting dispersions are particularly well suited for use in continuous polymerization procedures that can be carried out in coils, tubes, and elongated vessels adapted for continuously introducing the thickened dispersions into one end and for continuously withdrawing the mass of polymer beads from the other end. The polymerization step is also practiced in batch manner.

The order of the addition of the constituents to the polymerization usually is not critical, but beneficially it is more convenient to add to a vessel the water, dispersing agent, and incorporated the oil-soluble catalyst to the monomer mixture, and subsequently add with agitation the monomer phase to the water phase.

The following is an example illustrating a procedure for preparing the cross-linked polymeric microbeads coated with slip agent. In this example, the polymer is polystyrene cross-linked with divinylbenzene. The microbeads have a coating of silica. The microbeads are prepared by a procedure in which monomer droplets containing an initiator are sized and heated to give solid polymer spheres of the same size as the monomer droplets. A water phase is prepared by combining 7 liters of distilled water, 1.5 g potassium dichromate (polymerization inhibitor for the aqueous phase), 250 g polymethylaminoethanol adipate (promoter), and 350 g LUDOX (a colloidal suspension containing 50% silica sold by DuPont). A monomer phase is prepared by combining 3317 g styrene, 1421 g divinylbenzene (55% active cross-linking agent; other 45% is ethyl vinyl benzene which forms part of the styrene polymer chain) and 45 g VAZO 52 (a monomer-soluble initiator sold by DuPont). The mixture is passed through a homogenizer to obtain 5 micron droplets. The suspension is heated overnight at 52° C. to give 4.3 kg of generally spherical microbeads having an average diameter of about 5  $\mu\text{m}$  with narrow size distribution (about 2–10  $\mu\text{m}$  size distribution). The mol proportion of styrene and ethyl vinyl benzene to divinylbenzene is about 6.1%. The concentration of divinylbenzene can be adjusted up or down to result in about 2.5–50% (preferably 10–40%) cross-linking by the active cross-linker. Of course, monomers other than styrene and divinylbenzene can be used in similar suspension polymerization processes known in the art. Also, other initiators and promoters may be used as known in the art. Also, slip agents other than silica may also be used. For example, a number of LUDOX colloidal silicas are available from DuPont. LEPANDIN colloidal alumina is available from Degussa. NALCOAG colloidal silicas are available from Nalco, and tin oxide and titanium oxide are also available from Nalco.

Normally, for the polymer to have suitable physical properties such as resiliency, the polymer is cross-linked. In the case of styrene cross-linked with divinylbenzene, the polymer is 2.5–50% cross-linked, preferably 20–40% cross-linked. By percent cross-linked, it is meant the mol % of cross-linking agent based on the amount of primary monomer. Such limited cross-linking produces microbeads which are sufficiently coherent to remain intact during orientation of the continuous polymer. Beads of such cross-linking are also resilient so that when they are deformed (flattened) during orientation by pressure from the matrix polymer on opposite sides of the microbeads, they subsequently resume their normal spherical shape to produce the largest possible voids around the microbeads to thereby produce articles with less density.

The microbeads are referred to herein as having a coating of a "slip agent". By this term it is meant that the friction at the surface of the microbeads is greatly reduced. Actually, it is believed this is caused by the silica acting as miniature ball bearings at the surface. Slip agent may be formed on the surface of the microbeads during their formation by including it in the suspension polymerization mix.

Microbead size is regulated by the ratio of silica to monomer. For example, the following ratios produce the indicated size microbead:

| Microbead Size, $\mu\text{m}$ | Monomer, Parts by Wt. | Slip Agent (Silica) Parts by Wt. |
|-------------------------------|-----------------------|----------------------------------|
| 2                             | 10.4                  | 1                                |
| 5                             | 27.0                  | 1                                |
| 20                            | 42.4                  | 1                                |

10 The microbeads of cross-linked polymer range in size from 0.1–50 microns, and are present in an amount of 5–50% by weight based on the weight of the polyester. Microbeads of polystyrene should have a Tg of at least 20° C. higher than the Tg of the continuous matrix polymer and are hard compared to the continuous matrix polymer.

15 Elasticity and resiliency of the microbeads generally result in increased voiding, and it is preferred to have the Tg of the microbeads as high above that of the matrix polymer as possible to avoid deformation during orientation. It is not believed that there is a practical advantage to cross-linking above the point of resiliency and elasticity of the microbeads.

20 The microbeads of cross-linked polymers are at least partially bordered by voids. The void space in the supports should occupy 2–60%, preferably 30–50%, by volume of the shaped article. Depending on the manner in which the supports are made, the voids may completely encircle the microbeads, e.g., a void may be in the shape of a doughnut (or flattened doughnut) encircling a microbead, or the voids may only partially border the microbeads, e.g., a pair of voids may border a microbead on opposite sides.

25 During stretching, the voids assume characteristic shapes from the balanced biaxial orientation of paperlike films to the uniaxial orientation of microvoided/satinlike fibers. Balanced microvoids are largely circular in the plane of orientation, while fiber microvoids are elongated in the direction of the fiber axis. The size of the microvoids and the ultimate physical properties depend upon the degree and balance of the orientation, temperature and rate of stretching, crystallization kinetics, the size distribution of the microbeads, and the like.

30 The shaped articles and supports according to this invention are prepared by:

- 35 forming a mixture of molten continuous matrix polymer and cross-linked polymer wherein the cross-linked polymer is a multiplicity of microbeads uniformly dispersed throughout the matrix polymer, the matrix polymer being as described hereinbefore, the cross-linked polymer microbeads being as described hereinbefore,
- 40 forming a shaped article from the mixture by extrusion, casting or molding,
- 45 orienting the article by stretching to form microbeads of cross-linked polymer uniformly distributed throughout the article and voids at least partially bordering the microbeads on sides thereof in the direction, or directions of orientation.

50 The mixture may be formed by forming a melt of the matrix polymer and mixing therein the cross-linked polymer. The cross-linked polymer may be in the form of solid or semisolid microbeads. Due to the incompatibility between the matrix polymer and cross-linked polymer, there is no attraction or adhesion between them, and they become uniformly dispersed in the matrix polymer upon mixing.

55 When the microbeads have become uniformly dispersed in the matrix polymer, a shaped article is formed by processes such as extrusion, casting, or molding. Examples of

extrusion or casting would be extruding or casting a film or sheet, and an example of molding would be injection or reheat blow-molding a bottle. Such forming methods are well known in the art. If sheets or film material are cast or extruded, it is important that such article be oriented by stretching, at least in one direction. Methods of unilaterally or bilaterally orienting sheet or film material are well known in the art. Basically, such methods comprise stretching the sheet or film at least in the machine or longitudinal direction after it is cast or extruded an amount of about 1.5–10 times its original dimension. Such sheet or film may also be stretched in the transverse or cross-machine direction by apparatus and methods well known in the art, in amounts of generally 1.5–10 (usually 3–4 for polyesters and 6–10 for polypropylene) times the original dimension. Such apparatus and methods are well known in the art and are described in such U.S. Pat. No. 3,903,234.

The voids, or void spaces, referred to herein surrounding the microbeads are formed, as the continuous matrix polymer is stretched at a temperature above the  $T_g$  of the matrix polymer. The microbeads of cross-linked polymer are relatively hard compared to the continuous matrix polymer. Also, due to the incompatibility and immiscibility between the microbead and the matrix polymer, the continuous matrix polymer slides over the microbeads as it is stretched, causing voids to be formed at the sides in the direction or directions of stretch, which voids elongate as the matrix polymer continues to be stretched. Thus, the final size and shape of the voids depends on the direction(s) and amount of stretching. If stretching is only in one direction, microvoids will form at the sides of the microbeads in the direction of stretching. If stretching is in two directions (bidirectional stretching), in effect such stretching has vector components extending radially from any given position to result in a doughnut-shaped void surrounding each microbead.

The preferred preform stretching operation simultaneously opens the microvoids and orients the matrix material. The final product properties depend on and can be controlled by stretching time-temperature relationships and on the type and degree of stretch. For maximum opacity and texture, the stretching is done just above the glass transition temperature of the matrix polymer. When stretching is done in the neighborhood of the higher glass transition temperature, both phases may stretch together and opacity decreases. In the former case, the materials are pulled apart, a mechanical anticompatibilization process. Two examples are high-speed melt spinning of fibers and melt blowing of fibers and films to form nonwoven/spun-bonded products. In summary, the scope of this invention includes the complete range of forming operations just described.

In general, void formation occurs independent of, and does not require, crystalline orientation of the matrix polymer. Opaque, microvoided films have been made in accordance with the methods of this invention using completely amorphous, noncrystallizing copolymers as the matrix phase. Crystallizable/orientable (strain hardening) matrix materials are preferred for some properties like tensile strength and barrier. On the other hand, amorphous matrix materials have special utility in other areas like tear resistance and heat sealability. The specific matrix composition can be tailored to meet many product needs. The complete range from crystalline to amorphous matrix polymer is part of the invention.

The thick preferred embodiment of a translucent polymer base for the photographic element of this invention is an integral composite multilayer biaxially oriented polyolefin

sheet. Any suitable biaxially oriented polyolefin sheet may be used for the base of the invention. Microvoided biaxially oriented sheets are preferred and are conveniently manufactured by coextrusion of the core and surface layers, followed by biaxial orientation, whereby voids are formed around void-initiating material contained in the core layer.

The percent solid density should be between 45% and 100%, preferably between 80% and 100%. As the percent solid density becomes less than 67%, the composite sheet becomes less manufacturable due to a drop in tensile strength, and it becomes more susceptible to physical damage such as stress fracturing of the skin layer which will reduce the commercial value of an image.

The thickness of each of the voided core layers is preferably between 10 and 60  $\mu\text{m}$ . Manufacturing a voided layer less than 10  $\mu\text{m}$  is very difficult. Above 60  $\mu\text{m}$ , the structure becomes more susceptible to physical damage caused by stresses encountered when the photographic element is bent. Such stresses are encountered when photographic images are viewed and handled by the consumer.

The thickness of the upper layer (the layer between the photosensitive layer and the voided layer) is preferably between 1 and 15  $\mu\text{m}$ . Below 1  $\mu\text{m}$  in thickness, the microvoided sheet becomes difficult to manufacture as the limits of a biaxially oriented layer are reached. Above 15  $\mu\text{m}$ , little improvement is seen in the optical performance of the layer. The thickness of the layer adjacent and below the microvoided layer is preferably between 2 and 15  $\mu\text{m}$ . For the same reasons, manufacturing outside this range can either cause manufacturing problems or does not improve the optical performance of the photographic support.

The bending stiffness of the sheet can be measured by using the LORENTZEN & WETTRE STIFFNESS TESTER, MODEL 16D. The output from this instrument is the force, in millinewtons, required to bend the cantilevered, unclamped end of a clamped sample 20 mm long and 38.1 mm wide at an angle of 15 degrees from the unloaded position. A typical range of stiffness that is suitable for display material is 120 to 300 millinewtons. A stiffness greater than at least 120 millinewtons is required, as the imaging support begins to lose commercial value below that number. Further, imaging supports with stiffness less than 120 millinewtons are difficult to transport in photofinishing equipment.

"Void" is used herein to mean devoid of added solid and liquid matter, although it is likely the "voids" contain gas. The void-initiating particles which remain in the finished packaging sheet core should be from 0.1 to 10  $\mu\text{m}$  in diameter, preferably round in shape, to produce voids of the desired shape and size. The size of the void is also dependent on the degree of orientation in the machine and transverse directions. Ideally, the void would assume a shape which is defined by two opposed and edge contacting concave disks. In other words, the voids tend to have a lens-like or biconvex shape. The voids are oriented so that the two major dimensions are aligned with the machine and transverse directions of the sheet. The Z-direction axis is a minor dimension and is roughly the size of the cross diameter of the voiding particle. The voids generally tend to be closed cells and, thus, there is virtually no path open from one side of the voided-core to the other side through which gas or liquid can traverse.

The void-initiating material may be selected from a variety of materials and should be present in an amount of about 5–50% by weight based on the weight of the core matrix polymer. Preferably, the void-initiating material comprises a polymeric material. When a polymeric material is

used, it may be a polymer that can be melt-mixed with the polymer from which the core matrix is made and be able to form dispersed spherical particles as the suspension is cooled down. Examples of this would include nylon dispersed in polypropylene, polybutylene terephthalate in polypropylene, or polypropylene dispersed in polyethylene terephthalate. If the polymer is preshaped and blended into the matrix polymer, the important characteristic is the size and shape of the particles. Spheres are preferred and they can be hollow or solid. These spheres may be made from cross-linked polymers which are members selected from the group consisting of an alkenyl aromatic compound having the general formula  $\text{Ar}-\text{C}(\text{R})=\text{CH}_2$ , wherein Ar represents an aromatic hydrocarbon radical, or an aromatic halohydrocarbon radical of the benzene series and R is hydrogen or the methyl radical; acrylate-type monomers include monomers of the formula  $\text{CH}_2=\text{C}(\text{R}')-\text{C}(\text{O})(\text{OR})$  wherein R is selected from the group consisting of hydrogen and an alkyl radical containing from about 1 to 12 carbon atoms and R' is selected from the group consisting of hydrogen and methyl; copolymers of vinyl chloride and vinylidene chloride, acrylonitrile and vinyl chloride, vinyl bromide, vinyl esters having formula  $\text{CH}_2=\text{CH}(\text{O})\text{COR}$ , wherein R is an alkyl radical containing from 2 to 18 carbon atoms; acrylic acid, methacrylic acid, itaconic acid, citraconic acid, maleic acid, fumaric acid, oleic acid, vinylbenzoic acid; the synthetic polyester resins which are prepared by reacting terephthalic acid and dialkyl terephthalates or ester-forming derivatives thereof, with a glycol of the series  $\text{HO}(\text{CH}_2)_n\text{OH}$  wherein n is a whole number within the range of 2-10 and having reactive olefinic linkages within the polymer molecule, the above-described polyesters which include copolymerized therein up to 20 percent by weight of a second acid or ester thereof having reactive olefinic unsaturation and mixtures thereof, and a cross-linking agent selected from the group consisting of divinylbenzene, diethylene glycol dimethacrylate, diallyl fumarate, diallyl phthalate, and mixtures thereof.

Examples of typical monomers for making the cross-linked polymer include styrene, butyl acrylate, acrylamide, acrylonitrile, methyl methacrylate, ethylene glycol dimethacrylate, vinyl pyridine, vinyl acetate, methyl acrylate, vinylbenzyl chloride, vinylidene chloride, acrylic acid, divinylbenzene, acrylamidomethylpropane sulfonic acid, vinyl toluene, etc. Preferably, the cross-linked polymer is polystyrene or poly(methyl methacrylate). Most preferably, it is polystyrene, and the cross-linking agent is divinylbenzene.

Processes well known in the art yield nonuniformly sized particles, characterized by broad particle size distributions. The resulting beads can be classified by screening the beads spanning the range of the original distribution of sizes. Other processes such as suspension polymerization and limited coalescence directly yield very uniformly sized particles.

The void-initiating materials may be coated with agents to facilitate voiding. Suitable agents or lubricants include colloidal silica, colloidal alumina, and metal oxides such as tin oxide and aluminum oxide. The preferred agents are colloidal silica and alumina, most preferably, silica. The cross-linked polymer having a coating of an agent may be prepared by procedures well known in the art. For example, conventional suspension polymerization processes wherein the agent is added to the suspension is preferred. As the agent, colloidal silica is preferred.

The void-initiating particles can also be inorganic spheres, including solid or hollow glass spheres, metal or ceramic beads or inorganic particles such as clay, talc,

barium sulfate, and ium carbonate. The important thing is that the material does not chemically react with the core matrix polymer to cause one or more of the following problems: (a) alteration of the crystallization kinetics of the matrix polymer, making it difficult to orient, (b) destruction of the core matrix polymer, (c) destruction of the void-initiating particles, (d) adhesion of the void-initiating particles to the matrix polymer, or (e) generation of undesirable reaction products, such as toxic or high color moieties. The void-initiating material should not be photographically active or degrade the performance of the photographic element in which the biaxially oriented polyolefin sheet is utilized.

For the biaxially oriented sheet, suitable classes of thermoplastic polymers of the preferred composite sheet comprise polyolefins. Suitable polyolefins include polypropylene, polyethylene, polymethylpentene, polystyrene, polybutylene, and mixtures thereof. Polyolefin copolymers, including copolymers of propylene and ethylene such as hexene, butene, and octene, are also useful. Polypropylene and polyethylene are preferred, because they are low in cost and have desirable strength properties. Further, current light sensitive silver halide coatings have been optimized to adhere to polyethylene.

The nonvoided skin layers of the composite sheet can be made of the same polymeric materials as listed above for the voided core matrix. The composite sheet can be made with skin(s) of the same polymeric material as the core matrix, or it can be made with skin(s) of different polymeric composition than the core matrix.

The total thickness of the topmost skin layer should be between 0.20  $\mu\text{m}$  and 1.5  $\mu\text{m}$ , preferably between 0.5 and 1.0  $\mu\text{m}$ . Below 0.5  $\mu\text{m}$  any inherent nonplanarity in the coextruded skin layer may result in unacceptable color variation. At skin thickness greater than 1.5  $\mu\text{m}$ , there is a reduction in the photographic optical properties such as image resolution. At thickness greater than 1.5  $\mu\text{m}$ , there is also a greater material volume to filter for contamination such as clumps or poor color pigment dispersion.

Addenda may be added to the topmost skin layer to change the color of the imaging element. For photographic use, a white base with a slight bluish tinge is preferred. The addition of the slight bluish tinge may be accomplished by any process which is known in the art including the machine blending of color concentrate prior to extrusion and the melt extrusion of blue colorants that have been preblended at the desired blend ratio. Colored pigments that can resist extrusion temperatures greater than 320° C. are preferred, as temperatures greater than 320° C. are necessary for coextrusion of the skin layer. Blue colorants used in this invention may be any colorant that does not have an adverse impact on the imaging element. Preferred blue colorants include Phthalocyanine blue pigments, Cromophthal blue pigments, Irgazin blue pigments, and Irgalite organic blue pigments. Optical brightener may also be added to the skin layer to absorb UV energy and emit light largely in the blue region.

Additional addenda may be added to the core matrix and/or to the skins to improve the optical properties such as image sharpness, opacity, and whiteness of these sheets. This would also include adding fluorescing agents which absorb energy in the UV region and emit light largely in the blue region or other additives which would improve the physical properties of the sheet or the manufacturability of the sheet.

The coextrusion, quenching, orienting, and heat setting of these composite sheets may be effected by any process

which is known in the art for producing oriented sheet, such as by a flat sheet process or a bubble or tubular process. The flat sheet process involves extruding the blend through a slit die and rapidly quenching the extruded web upon a chilled casting drum so that the core matrix polymer component of the sheet and the skin component(s) are quenched below their glass solidification temperature. The quenched sheet is then biaxially oriented by stretching in mutually perpendicular directions at a temperature above the glass transition temperature and below the melting temperature of the matrix polymers. The sheet may be stretched in one direction and then in a second direction or may be simultaneously stretched in both directions. After the sheet has been stretched, it is heat set by heating to a temperature sufficient to crystallize or anneal the polymers, while restraining to some degree the sheet against retraction in both directions of stretching.

The composite sheet, while described as having preferably at least three layers of a microvoided core and a skin layer on each side, may also be provided with additional layers that may serve to change the properties of the biaxially oriented sheet. Biaxially oriented sheets could be formed with surface layers that would provide an improved adhesion the support and photographic element. The biaxially oriented extrusion could be carried out with as many as 10 layers if desired to achieve some particular desired property.

These composite sheets may be coated or treated after the coextrusion and orienting process or between casting and full orientation with any number of coatings which may be used to improve the properties of the sheets including printability, to provide a vapor barrier, to make them heat sealable, or to improve the adhesion to the support or to the photosensitive layers. Examples of this would be acrylic coatings for printability and coating polyvinylidene chloride for heat seal properties. Further examples include flame, plasma, or corona discharge treatment to improve printability or adhesion.

By having at least one nonvoided skin on the microvoided core, the tensile strength of the sheet is increased and makes it more manufacturable. It allows the sheets to be made at wider widths and higher draw ratios than when sheets are made with all layers voided. Coextruding the layers further simplifies the manufacturing process.

An example of a preferred multilayer biaxially oriented translucent base material is as follows where the photographic element is coated on the polyethylene top layer:

---

Polyethylene skin layer with blue tint  
 Polypropylene with optical brightener  
 Voided polypropylene core  
 Polypropylene skin layer

---

As used herein, the phrase "photographic element" is an imaging element that utilizes photosensitive silver halide in the formation of images. The photographic elements can be black-and-white, single color elements or multicolor elements. Multicolor elements contain image dye-forming units sensitive to each of the three primary regions of the spectrum. Each unit can comprise a single emulsion layer or multiple emulsion layers sensitive to a given region of the spectrum. The layers of the element, including the layers of the image-forming units, can be arranged in various orders as known in the art. In an alternative format, the emulsions sensitive to each of the three primary regions of the spectrum can be disposed as a single segmented layer.

For the display material of this invention, at least one image layer comprises at least one imaging layer containing silver halide and a dye forming coupler located on the topside of said imaging element is preferred. When an increase in dye density is required, one imaging layer containing silver halide and a dye forming coupler located on the topside and bottom side of said imaging element are preferred. Coating the imaging layer containing silver halide and a dye forming coupler on both sides of the support of this invention allows for a 50-second developer time which maintains the efficiency of the image development process while increasing dye density of the display image.

The photographic emulsions useful for this invention are generally prepared by precipitating silver halide crystals in a colloidal matrix by methods conventional in the art. The colloid is typically a hydrophilic film forming agent such as gelatin, alginic acid, or derivatives thereof.

The crystals formed in the precipitation step are washed and then chemically and spectrally sensitized by adding spectral sensitizing dyes and chemical sensitizers, and by providing a heating step during which the emulsion temperature is raised, typically from 40° C. to 70° C., and maintained for a period of time. The precipitation and spectral and chemical sensitization methods utilized in preparing the emulsions employed in the invention can be those methods known in the art.

Chemical sensitization of the emulsion typically employs sensitizers such as sulfur-containing compounds, e.g., allyl isothiocyanate, sodium thiosulfate and allyl thiourea; reducing agents, e.g., polyamines and stannous salts; noble metal compounds, e.g., gold, platinum; and polymeric agents, e.g., polyalkylene oxides. As described, heat treatment is employed to complete chemical sensitization. Spectral sensitization is effected with a combination of dyes, which are designed for the wavelength range of interest within the visible or infrared spectrum. It is known to add such dyes both before and after heat treatment.

After spectral sensitization, the emulsion is coated on a support. Various coating techniques include dip coating, air knife coating, curtain coating, and extrusion coating.

The silver halide emulsions utilized in this invention may be comprised of any halide distribution. Thus, they may be comprised of silver chloride, silver bromide, silver bromochloride, silver chlorobromide, silver iodochloride, silver iodobromide, silver bromoiodochloride, silver chloroiodobromide, silver iodobromochloride, and silver iodochlorobromide emulsions. It is preferred, however, that the emulsions be predominantly silver chloride emulsions. By predominantly silver chloride, it is meant that the grains of the emulsion are greater than about 50 mole percent silver chloride. Preferably, they are greater than about 90 mole percent silver chloride and optimally greater than about 95 mole percent silver chloride.

The silver halide emulsions can contain grains of any size and morphology. Thus, the grains may take the form of cubes, octahedrons, cubo-octahedrons, or any of the other naturally occurring morphologies of cubic lattice type silver halide grains. Further, the grains may be irregular such as spherical grains or tabular grains. Grains having a tabular or cubic morphology are preferred.

The photographic elements of the invention may utilize emulsions as described in *The Theory of the Photographic Process*, Fourth Edition, T. H.

James, Macmillan Publishing Company, Inc., 1977, pages 151-152. Reduction sensitization has been known to improve the photographic sensitivity of silver halide emulsions. While reduction sensitized silver halide emulsions

generally exhibit good photographic speed, they often suffer from undesirable fog and poor storage stability.

Reduction sensitization can be performed intentionally by adding reduction sensitizers, chemicals which reduce silver ions to form metallic silver atoms, or by providing a reducing environment such as high pH (excess hydroxide ion) and/or low pAg (excess silver ion). During precipitation of a silver halide emulsion, unintentional reduction sensitization can occur when, for example, silver nitrate or alkali solutions are added rapidly or with poor mixing to form emulsion grains. Also, precipitation of silver halide emulsions in the presence of ripeners (grain growth modifiers) such as thioethers, selenoethers, thioureas, or ammonia tends to facilitate reduction sensitization.

Examples of reduction sensitizers and environments which may be used during precipitation or spectral/chemical sensitization to reduction sensitize an emulsion include ascorbic acid derivatives; tin compounds; polyamine compounds; and thiourea dioxide-based compounds described in U.S. Pat. Nos. 2,487,850; 2,512,925; and British Patent 789,823. Specific examples of reduction sensitizers or conditions, such as dimethylamineborane, stannous chloride, hydrazine, high pH (pH 8–11), and low pAg (pAg 1–7) ripening are discussed by S. Collier in *Photographic Science and Engineering*, 23, 113 (1979). Examples of processes for preparing intentionally reduction sensitized silver halide emulsions are described in EP 0 348 934 A1 (Yamashita), EP 0 369 491 (Yamashita), EP 0 371 388 (Ohashi), EP 0 396 424 A1 (Takada), EP 0 404 142 A1 (Yamada), and EP 0 435 355 A1 (Makino).

The photographic elements of this invention may use emulsions doped with Group VIII metals such as iridium, rhodium, osmium, and iron as described in *Research Disclosure*, September 1994, Item 36544, Section I, published by Kenneth Mason Publications, Ltd., Dudley Annex, 12a North Street, Emsworth, Hampshire PO10 7DQ, ENGLAND. Additionally, a general summary of the use of iridium in the sensitization of silver halide emulsions is contained in Carroll, "Iridium Sensitization: A Literature Review," *Photographic Science and Engineering*, Vol. 24, No. 6, 1980. A method of manufacturing a silver halide emulsion by chemically sensitizing the emulsion in the presence of an iridium salt and a photographic spectral sensitizing dye is described in U.S. Pat. No. 4,693,965. In some cases, when such dopants are incorporated, emulsions show an increased fresh fog and a lower contrast sensitometric curve when processed in the color reversal E-6 process as described in *The British Journal of Photography Annual*, 1982, pages 201–203.

A typical multicolor photographic element of the invention comprises the invention laminated support bearing a cyan dye image-forming unit comprising at least one red-sensitive silver halide emulsion layer having associated therewith at least one cyan dye-forming coupler; a magenta image-forming unit comprising at least one green-sensitive silver halide emulsion layer having associated therewith at least one magenta dye-forming coupler; and a yellow dye image-forming unit comprising at least one blue-sensitive silver halide emulsion layer having associated therewith at least one yellow dye-forming coupler. The element may contain additional layers, such as filter layers, interlayers, overcoat layers, subbing layers, and the like. The support of the invention may also be utilized for black-and-white photographic print elements.

The photographic elements may also contain a transparent magnetic recording layer such as a layer containing magnetic particles on the underside of a transparent support, as

in U.S. Pat. Nos. 4,279,945 and 4,302,523. Typically, the element will have a total thickness (excluding the support) of from about 5 to about 30  $\mu\text{m}$ .

In the following Table, reference will be made to (1) *Research Disclosure*, December 1978, Item 17643, (2) *Research Disclosure*, December 1989, Item 308119, and (3) *Research Disclosure*, September 1994, Item 36544, all published by Kenneth Mason Publications, Ltd., Dudley Annex, 12a North Street, Emsworth, Hampshire PO10 7DQ, ENGLAND. The Table and the references cited in the Table are to be read as describing particular components suitable for use in the elements of the invention. The Table and its cited references also describe suitable ways of preparing, exposing, processing and manipulating the elements, and the images contained therein.

| Reference | Section                                             | Subject Matter                                                                 |
|-----------|-----------------------------------------------------|--------------------------------------------------------------------------------|
| 1         | I, II                                               | Grain composition, morphology and preparation.                                 |
| 2         | I, II, IX, X, XI, XII, XIV, XV I, II, III, IX A & B | Emulsion preparation including hardeners, coating aids, addenda, etc.          |
| 3         | III, IV                                             | Chemical sensitization and spectral sensitization/ desensitization             |
| 2         | III, IV                                             | UV dyes, optical brighteners, luminescent dyes                                 |
| 3         | IV, V                                               |                                                                                |
| 1         | V                                                   |                                                                                |
| 2         | V                                                   |                                                                                |
| 3         | VI                                                  |                                                                                |
| 1         | VI                                                  |                                                                                |
| 2         | VI                                                  | Antifoggants and stabilizers                                                   |
| 3         | VII                                                 |                                                                                |
| 1         | VIII                                                |                                                                                |
| 2         | VIII, XIII, XVI                                     | Absorbing and scattering materials; Antistatic layers; matting agents          |
| 3         | VIII, IX C & D                                      |                                                                                |
| 1         | VII                                                 | Image-couplers and image-modifying couplers; Dye stabilizers and hue modifiers |
| 2         | VII                                                 |                                                                                |
| 3         | X                                                   |                                                                                |
| 1         | XVII                                                |                                                                                |
| 2         | XVII                                                | Supports                                                                       |
| 3         | XV                                                  |                                                                                |
| 3         | XI                                                  | Specific layer arrangements                                                    |
| 3         | XII, XIII                                           | Negative working emulsions; Direct positive emulsions                          |
| 2         | XVIII                                               | Exposure                                                                       |
| 3         | XVI                                                 |                                                                                |
| 1         | XIX, XX                                             |                                                                                |
| 2         | XIX, XX, XXII                                       | Chemical processing; Developing agents                                         |
| 3         | XVIII, XIX, XX                                      |                                                                                |
| 3         | XIV                                                 | Scanning and digital processing procedures                                     |

The photographic elements can be exposed with various forms of energy which encompass the ultraviolet, visible, and infrared regions of the electromagnetic spectrum, as well as with electron beam, beta radiation, gamma radiation, X ray, alpha particle, neutron radiation, and other forms of corpuscular and wavelike radiant energy in either noncoherent (random phase) forms or coherent (in phase) forms, as produced by lasers. When the photographic elements are intended to be exposed by X rays, they can include features found in conventional radiographic elements.

For the preferred reflective/transmission display material of this invention wherein said imaging element comprises at least one dye forming layer comprising silver halide and dye forming coupler on both sides of said translucent polymer sheet, the imaging elements of this invention are preferably exposed by means of a collimated beam, to form a latent

image, and then processed to form a visible image, preferably by other than heat treatment. A collimated beam is preferred, as it allows for digital printing and simultaneous exposure of the imaging layer on the top and bottom side without significant internal light scatter. A preferred example of a collimated beam is a laser also known as light amplification by stimulated emission of radiation. The laser is preferred because this technology is used widely in a number of digital printing equipment types. Further, the laser provides sufficient energy to simultaneously expose the light sensitive silver halide coating on the top and bottom side of the display material of this invention without undesirable light scatter. Subsequent processing of the latent image into a visible image is preferably carried out in the known RA-4™ (Eastman Kodak Company) Process or other processing systems suitable for developing high chloride emulsions.

After processing and development of the photographic element of this invention, the photographic element may be used as a transmission display material for commercial and consumer use. Prior art transmission display materials for commercial use are typically large format (100 cm×200 cm) and are used in combination with a device that provides backlighting of the image. For home use by consumers, a display apparatus comprising a container provided with one side that is at least partially open or transparent, a light source adapted to provide light directed to the open or transparent side, means to suspend a photographic element is preferred. This display apparatus will allow high quality display images with a maintained dye hue angle to be viewed in the home. An example of consumer use of the photographic element of this invention in combination with the preferred display apparatus is desktop viewing of transmission images.

The following examples illustrate the practice of this invention. They are not intended to be exhaustive of all possible variations of the invention. Parts and percentages are by weight unless otherwise indicated.

## EXAMPLES

### Example 1

In this example, a nontransparent photographic display material with maintained hue angle was made by laminating a biaxially oriented polyolefin sheet to a photographic grade polyester sheet. The nontransparent display materials were then coated with a typical consumer silver halide emulsion. The biaxially oriented sheet of this example had levels of voiding selected to provide diffusion of the illuminating light source. The invention was compared to a prior art transmission display material with  $TiO_2$  in the base. In order to measure the dye hue angle change, the silver halide emulsion was also coated on a transparent polyester base without any white pigments. This example will show that the yellow, magenta, and cyan dye hue angles were maintained within  $+/-5$  degrees from the dyes coated on the transparent support, whereas the prior art transmission support with  $TiO_2$  had dye hue angles that were  $+/-10$  degrees from the dyes coated on the transparent support.

The following photographic transmission display material of the invention was prepared by extrusion laminating the following biaxially oriented polyolefin sheet to top side of a photographic grade polyester base:

#### Top Sheet (Emulsion side):

A composite sheet consisting of 5 layers identified as L1, L2, L3, L4, and L5. L1 is the thin colored layer on the top of the biaxially oriented sheet to which the photosensitive

silver halide layer was attached. L2 is the layer to which optical brightener was added. The optical brightener used was Hostalux KS manufactured by Ciba-Geigy. Photographic Grade Polyester Base:

A polyethylene terephthalate base 110  $\mu m$  thick that was transparent and gelatin coated and dried on both sides of the base. The polyethylene terephthalate base had a stiffness of 30 millinewtons in the machine direction and 40 millinewtons in the cross direction.

The top sheet used in this example was coextruded and biaxially oriented. The top sheet was melt extrusion laminated to the polyester base using a metallocene catalyzed ethylene plastomer (SLP 9088) manufactured by Exxon Chemical Corp. The metallocene catalyzed ethylene plastomer had a density of 0.900 g/cc and a melt index of 14.0.

The L3 layer for the biaxially oriented sheet is microvoided and further described in Table 2 where the refractive index and geometrical thickness is shown for measurements made along a single slice through the L3 layer; they do not imply continuous layers; a slice along another location would yield different but approximately the same thickness. The areas with a refractive index of 1.0 are voids that are filled with air and the remaining layers are polypropylene.

TABLE 1

| Sublayer of L3 | Refractive Index | Thickness, $\mu m$ |
|----------------|------------------|--------------------|
| 1              | 1.49             | 2.54               |
| 2              | 1                | 1.527              |
| 3              | 1.49             | 2.79               |
| 4              | 1                | 1.016              |
| 5              | 1.49             | 1.778              |
| 6              | 1                | 1.016              |
| 7              | 1.49             | 2.286              |
| 8              | 1                | 1.016              |
| 9              | 1.49             | 2.032              |
| 10             | 1                | 0.762              |
| 11             | 1.49             | 2.032              |
| 12             | 1                | 1.016              |
| 13             | 1.49             | 1.778              |
| 14             | 1                | 1.016              |
| 15             | 1.49             | 2.286              |

The structure of the invention was as follows:

---

|                                          |
|------------------------------------------|
| Polyethylene with blue tints             |
| Polypropylene with optical brightener    |
| Microvoided polypropylene                |
| Metallocene catalyzed ethylene plastomer |
| Gelatin sub coating layer                |
| Transparent polyester base               |
| Gelatin sub coating layer                |

---

The control used in this example is typical of prior art materials that use  $TiO_2$  as a diffuser of the illumination light source. The prior art material used in this example was Kodak Duratrans (Eastman Kodak Co.) which is a one side color silver halide coated polyester support that is 180  $\mu m$  thick. Coating format 1 was used to coat this support. The support is a clear gel subbed photographic grade polyester. The silver halide emulsion contains 200 mg/ $ft^2$  of rutile  $TiO_2$  in the bottom most gelatin layer.

Coating format 1 below was coated on a transparent photographic grade polyethylene terephthalate base to establish the native or inherent dye hue for coating format 1. The polyethylene terephthalate base was 110  $\mu m$  thick and gelatin subbed on both sides of the base. The polyethylene terephthalate base had a stiffness of 30 millinewtons in the machine direction and 40 millinewtons in the cross direction. The % transmission of the polyester base material was 96%.

**31**

Coating format 1 was utilized to prepare photographic transmission display materials and was coated on the L1 polyethylene layer on the top biaxially oriented sheet.

|         | Coating Format 1           | Laydown mg/m <sup>2</sup> |    |
|---------|----------------------------|---------------------------|----|
| Layer 1 | <u>Blue Sensitive</u>      |                           |    |
|         | Gelatin                    | 1300                      | 5  |
|         | Blue sensitive silver      | 200                       | 10 |
|         | Y-1                        | 440                       |    |
|         | ST-1                       | 440                       |    |
|         | S-1                        | 190                       |    |
| Layer 2 | <u>Interlayer</u>          |                           |    |
|         | Gelatin                    | 650                       | 15 |
|         | SC-1                       | 55                        |    |
|         | S-1                        | 160                       |    |
| Layer 3 | <u>Green Sensitive</u>     |                           |    |
|         | Gelatin                    | 1100                      | 20 |
|         | Green sensitive silver     | 70                        |    |
|         | M-1                        | 270                       |    |
|         | S-1                        | 75                        |    |
|         | S-2                        | 32                        |    |
|         | ST-2                       | 20                        |    |
|         | ST-3                       | 165                       |    |
|         | ST-4                       | 530                       |    |
| Layer 4 | <u>UV Interlayer</u>       |                           |    |
|         | Gelatin                    | 635                       | 25 |
|         | UV-1                       | 30                        |    |
|         | UV-2                       | 160                       |    |
|         | SC-1                       | 50                        |    |
|         | S-3                        | 30                        |    |
|         | S-1                        | 30                        |    |
| Layer 5 | <u>Red Sensitive Layer</u> |                           |    |
|         | Gelatin                    | 1200                      | 30 |
|         | Red sensitive silver       | 170                       |    |
|         | C-1                        | 365                       |    |
|         | S-1                        | 360                       |    |
|         | UV-2                       | 235                       |    |
|         | S-4                        | 30                        |    |
|         | SC-1                       | 3                         |    |
| Layer 6 | <u>UV Overcoat</u>         |                           |    |
|         | Gelatin                    | 440                       | 35 |
|         | UV-1                       | 20                        |    |
|         | UV-2                       | 110                       |    |
|         | SC-1                       | 30                        |    |
|         | S-3                        | 20                        |    |
|         | S-1                        | 20                        |    |
| Layer 7 | <u>SOC</u>                 |                           |    |
|         | Gelatin                    | 490                       | 40 |
|         | SC-1                       | 17                        |    |
|         | SiO <sub>2</sub>           | 200                       |    |
|         | Surfactant                 | 2                         |    |

APPENDIX

Y-1

55



UV-1



UV-2

ST-1 = N-tert-butylacrylamide / n-butyl acrylate copolymer (50:50)  
 S-1 = dibutyl phthalate

65 S-3 = 1,4-Cyclohexyldimethylene bis(2-ethylhexanoate)

**32**

-continued

SC-1



M-1



S-2 = diundecyl phthalate

ST-2



ST-3



ST-4



UV-1



UV-2



-continued



The display materials of this example were printed with test images using a three color (red, green, and blue) laser sensitometer. The display support was measured for spectral transmission using an X-Rite Model 310 photographic densitometer. The display materials were also measured in transmission for  $L^*$ ,  $a^*$ , and  $b^*$  using a Hunter spectrophotometer, CIE system, using procedure D6500. In the transmission mode, a qualitative assessment was made as to the amount of illuminating backlighting show through. A substantial amount of show through would be considered undesirable, as the filaments of the lights would interfere with the display materials image. The data for invention are listed in Table 2 below.

TABLE 2

| Measure                            | Invention | Prior Art Transmission Material | Dyes Coated on Transparent Support |
|------------------------------------|-----------|---------------------------------|------------------------------------|
| % Transmission                     | 40%       | 42%                             | 96%                                |
| Cyan hue angle                     | 205       | 196                             | 210                                |
| Magenta hue angle                  | 330       | 337                             | 329                                |
| Yellow hue angle                   | 101       | 96                              | 98                                 |
| Illuminating Backlight Showthrough | None      | Slight                          | Heavy                              |

The invention transmission display support coated with the light sensitive silver halide coating format of this example exhibits all the properties needed for a photographic transmission display material. Further, the photographic transmission display material of this invention has many advantages over the prior art transmission display material which is typical of prior art transmission display materials with incorporated  $TiO_2$ . The voided and non-voided layers of the invention have levels of optical brightener and colorants adjusted to provide optimum optical properties for control of  $L^*$ , opacity, and filament show through. Because the native yellowness of coating format 1 was offset by the blue tinting in L1 in the invention, the density minimum areas for the invention were neutral white compared to the yellowness of the control material producing a perceptually preferred display material. The % transmission for the invention (40%) was roughly equivalent to

the prior art materials (42%) without the expensive use of  $TiO_2$  as an illumination light source diffuser. The invention did not have any illuminating light source show through compared to a slight show through for the prior art material.

5 The hue angle of the yellow, magenta, and cyan dye set of coating format 1 was changed less with a translucent support containing no white pigments compared to the control sample which had incorporated  $TiO_2$ . The dye hue angle for the coating format 1 yellow dye coated on a transparent support was 98 degrees. The same yellow dye coated on the prior art material produced a yellow dye hue angle of 96 degrees, which translates into a red yellow. The yellow dye set in coating format 1, when coated on the translucent base of the invention, yielded a perceptually preferred yellow dye hue angle of 96 degrees, which translates into a green yellow. The green yellow, being perceptually preferred, produces a higher quality image than the control, and a yellow green will tend to draw more attention to the display material. The data above also show that the magenta dye hue angle changed only 1 degree with the invention compared to 8 degrees with the prior art transmission material. Similarly, the cyan dye hue angle changes only 5 degrees with the invention material, while it changes 14 degrees with the prior art transmission material.

In summary, the invention display materials only changes 25 the dye hue  $\pm 5$  degrees from the inherent dye hue of coating format 1 coated on a transparent support compared to the prior art materials which changed  $\pm 14$  degrees. The invention material did a much better job maintaining the dye hue of coating format 1 leading to a perceptually preferred image compared to the prior art display materials.

The invention has been described in detail with particular reference to certain preferred embodiments thereof, but it will be understood that variations and modifications can be effected within the spirit and scope of the invention.

35 What is claimed is:

1. A photographic element comprising a translucent base and a color forming layer comprising at least one silver halide emulsion layer and dye forming coupler, wherein said base comprises at least one polymer sheet comprising a 40 transparent polymer sheet containing voids, with the proviso that said translucent sheet is substantially free of white light reflecting pigments and wherein said translucent base has a light transmission of between 15% and 85%, wherein said translucent base comprises an integral composite coextruded biaxially oriented polyolefin sheet.

2. The photographic element of claim 1 wherein said translucent base is a laminate comprising a transparent polymer sheet having laminated thereto said translucent sheet, and said translucent sheet comprises said biaxially oriented polyolefin sheet.

50 3. The photographic element of claim 1 wherein said transparent polymer sheet comprises polyester polymer sheet.

4. The photographic element of claim 1 wherein said biaxially oriented polyolefin sheet comprises a multilayer coextruded sheet wherein at least one layer is voided.

5. The photographic element of claim 1 wherein said photographic element comprises at least one layer comprising light sensitive silver halide and a dye forming coupler on each side of said base.

60 6. The photographic element of claim 5 wherein said voided polyester sheet comprises a multilayer coextruded sheet wherein at least one layer is voided.

7. The photographic element of claim 1 wherein said light transmission is between 34 and 42%.

65 8. The photographic element of claim 1 wherein said element after exposure and development has a change in hue

**35**

angle of less than about 5 degrees from the hue angle of the same dye on a substantially transparent base.

9. The photographic element of claim 1 wherein said light transmission is between 85% and 40%.

10. The photographic element of claim 1 wherein the average void percentage of said transparent polymer is between 10% and 60% by volume.

11. The photographic element of claim 1 wherein the void initiating material in the voids of said base is not a pigmented material.

12. A display apparatus comprising a container provided with one side that is at least partially open or transparent, a light source adapted to provide light directed to the open or transparent side, means to suspend a photographic element comprising a base, a color layer formed by the reaction of at least one silver halide emulsion layer and dye forming coupler, wherein said base comprises a translucent polymer sheet comprising a transparent polymer containing voids, with the proviso that said translucent sheet is substantially free of white light reflecting pigments and said translucent sheet has a light transmission between 15% and 85% and is suspended in said one side that is at least partially open, wherein said translucent base comprises an integral composite coextruded biaxially oriented polyolefin sheet.

13. The display apparatus of claim 12 wherein said translucent base is a laminate comprising a transparent

**36**

polymer sheet having laminated thereto said translucent sheet, and said translucent sheet comprises a biaxially oriented polyolefin sheet.

14. The display apparatus of claim 12 wherein said translucent base consists of an integral composite coextruded biaxially oriented polyolefin sheet.

15. The display apparatus of claim 14 wherein said biaxially oriented polyolefin sheet comprises a multilayer coextruded sheet wherein at least one layer is voided.

16. The display apparatus of claim 13 wherein said light transmission is between 34 and 42%.

17. The display apparatus of claim 13 wherein said transparent polymer sheet comprises a polyester sheet.

18. The display apparatus of claim 13 wherein said element after exposure and development has a change in hue angle of less than about 5 degrees from the hue angle of the same dye on a substantially transparent base.

19. The display apparatus of claim 13 wherein said light transmission is between 85% and 40%.

20. The display apparatus of claim 12 wherein the average void percentage of said transparent polymer is between 10% and 60% by volume.

\* \* \* \* \*